

## UNITED STATES PATENT OFFICE

2,083,052

DENTAL ALLOY AND METHOD OF MAKING  
SAME

Edward L. Chott, Riverside, Ill.

No Drawing. Application April 24, 1935,  
Serial No. 17,931

3 Claims. (Cl. 75—173)

This invention relates to an alloy adaptable for use in dental amalgams and to a novel process of preparing such alloy in finely divided or comminuted particles which are annealed and treated in the manner hereinafter described. 5  
More particularly, my invention embodies a dental alloy which is composed of silver, tin and zinc which have been combined in carefully worked out and definite range of proportions. This alloy of my invention when finely comminuted and triturated with the proper proportion of mercury, results in a plastic mixture which will readily harden into a rigid metallic body in a relatively short time and to a hardness equal to that which will sustain a pressure considerably in excess of dental alloys prepared with presently known proportions and methods. 10

Most alloys used at present contain a large proportion of silver and have combined therewith a substantial amount of copper, it being understood and assumed by makers of dental alloys that copper is an essential ingredient and used for the presently assumed essential function of limiting and stabilizing the hardening of amalgam made with such alloys. It is also known that the copper content of dental alloys materially increases the discoloration and tarnishing of presently known alloys due to reactions thereof with the sulphur and other compounds contained in foods. The alloy of my invention and its method of preparation eliminates the use of copper and likewise eliminates its aforesaid undesirable characteristics, at the same time possessing the same properties of relatively quick hardening and limited but desirable degree of expansion and a hard tough resultant body which is free from cracks or pores. Various objects of my invention are set forth as follows. 25

An important object of my invention is the provision of a dental alloy composed of the proper proportions of silver and tin and a relatively small proportion of zinc which eliminates the necessity of the use of copper, at the same time having a relatively small but desirable amount of expansion upon setting, and which attains a hardness sufficient to sustain a pressure of approximately 3,500 pounds per square inch. 30

A further object of my invention is the provision of an alloy composed of proper proportions of silver, tin and zinc, and no copper whatever, which at the same time will not only have the desirable amount of expansion when setting, but which also has the important characteristic of 35

maintaining the natural color of the alloy and not susceptible to discoloration or tarnish when it has come in contact with sulphur and other numerous agents present in various foods. 40

A further important object of my invention is the provision of a dental alloy for use in dental amalgams which is composed of only silver, tin and zinc in predetermined range of proportions and which has a strong characteristic of maintaining its natural color as possessed by it before actual use, namely, avoiding tarnish and discoloration which are caused upon presently known dental alloys containing silver by sulphur and other agents found in food and in the atmosphere in the form of gaseous compounds. 45

A further object of my invention is the provision of an alloy which avoids the conventional use of copper, copper being considered as a necessary ingredient of presently known alloys, copper having undesirable characteristics of discoloration and tarnish and heretofore considered as a stabilizer to prevent over-expansion during setting and hardening, my said alloy being mixable with mercury to make a plastic mixture which will harden in a relatively short time to a degree measurable to withstand a pressure of approximately 3,500 pounds per square inch, and which has a desirable degree of expansion on setting sufficient to prevent leakage from within the tooth cavity into which the amalgam is inserted. 50

A further object of my invention is the provision of a novel process of preparing an alloy for use in a novel dental amalgam which comprises melting the component metals in a sealed furnace, thence pouring the same into moulds, then dividing the same into fine particles by chipping, shaving and crushing and then sealing and annealing the same to prevent contraction or over-expansion when the amalgam made from such alloy is fully set and to control the hardening time thereof, such annealing being accomplished by placing the alloy in small containers under vacuum and boiling for desired periods of time. 55

Another object of my invention is to overcome the undesirable characteristic brought about by the conventional use of copper, providing an alloy of finely divided particles which have been sieved or crushed to a small size so that one troy ounce will measure from 8 to 10 cubic centimeters and which will yield an amalgam providing a complete filling and sealing of the cavity without voids, cracks or channels, either in the amalgam body or between it and the tooth. 60

It is well known by those familiar with ordinary 65

and presently known dental alloys that such ordinary alloys contain copper as a base ingredient, it being the assumption that the copper has the property of preventing over-expansion of the alloy upon setting and thereby acting as a stabilizer. Because of the general use of copper as a basic ingredient in presently known alloys for making dental amalgam, all such alloys have the undesirable characteristic of quickly becoming tarnished and discolored due to the action of agents contained in foods, particularly sulphur, which in a very short time tarnishes the tooth filling to a dark and unnatural appearance, usually a bluish gray color. I have found after lengthy and repeated investigation that the use of copper can be entirely eliminated providing the proper proportions of the remaining ingredients specified hereinafter are combined in a manner and method which is novel in the art and which varies materially from presently known methods of preparing the dental alloy.

I first separate silver of a high degree of fineness (in a preferred proportion ranging from 71% to 78% of the total mass sought to be prepared) and melt the same in an electric or other suitable furnace, preferably of the induction type, so that during the melting process the alloy will be protected from contamination or oxidation. Tin of a proportion of from 21% to 28%, preferably 21.5% to 27.5%, and zinc of a proportion of less than one per cent and not less than  $\frac{1}{16}$  of one per cent or any zinc proportion between  $\frac{1}{16}$  of one per cent and 1%, is also melted in a suitable furnace in like manner and combined with the melted silver, whereafter I then pour the molten alloy into moulds, preferably round bars or tubes, and allow the same to cool and harden. I have found that while any preparation of the three ingredients herein stated within the ranges aforesaid is highly satisfactory, the most preferable proportions of tin is from 21.5% to 27% and of zinc from  $\frac{1}{16}$  of one per cent to and including 1%. Thereafter I cut the moulded bars or tubes into fine chips or shavings, either in a lathe, milling or filing machine. The resultant filings or shavings are then further reduced in size by sieving and crushing to a size so that from 8 to 10 cubic centimeters thereof will weigh one troy ounce.

The next step in my method of preparing my dental alloy is the annealing thereof which imparts properties thereto to control the setting and hardening time to prevent contraction and excessive expansion after the alloy is set in the tooth cavity. The first step in my annealing process is to pour the sieved and crushed alloy of the desired fineness into either glass or preferably metal tubes, the bottom of which tubes have been sealed with an air-tight cap and the upper end of said tube preferably having a screw capped

fitting with a valve therein. I then withdraw most of the air from each said tube by pumping the same out through aforesaid valve which will be closed against the entrance of air thereafter. I then place the tubes containing the alloy and in which partial vacuum is created into a tank of cold water, which water is slowly heated to the boiling point and left to boil for an interval of time. If the size of the alloy particles contained in the tube is slightly larger than those which I have specified in my preferred example, the duration of the boiling of such water during said annealing process should be proportionately longer. Further, the duration of the boiling time may also be gauged by the setting time required in order to obtain a fully annealed alloy which will retain its size after slight expansion (ranging from 3 to 13 microns) when setting in a tooth cavity.

I am aware that numerous details of proportion may be varied through a wide range without departing from the principles of this invention, and I therefore do not desire to limit the patent granted hereon otherwise than necessitated by the prior art.

I claim as my invention:

1. A comminuted ternary alloy for dental amalgams composed of from 71% to 78% silver and from 21% to 28% tin and 1% zinc and which has and will maintain its natural color and appearance, which will not have an excessive amount of expansion on setting; and which is uncontaminated due to maintenance thereof out of contact with the atmosphere during its melting, chipping, crushing and annealing steps.

2. An alloy for dental amalgams composed of from 72% to 78% silver and from 21.5% to 27.5% tin and  $\frac{1}{16}$  of one per cent to one per cent zinc, in finely divided form and annealed and which has the desirable characteristics of maintaining its natural color and avoiding discoloration when placed in contact with food agents and gaseous atmospheric compounds, and which when triturated will form a hard body equal to a hardness capable of sustaining a pressure of 3,500 pounds per square inch and which will not expand excessively or to great degree on setting.

3. The method of preparing an alloy for dental amalgams which comprises melting from 72 to 78 parts of silver; 21 to 27 parts of tin and zinc of from  $\frac{1}{16}$  to one percent; thence casting the same into relatively small moulds; thence comminuting the same into relatively fine particles; thence placing the comminuted alloy into airtight containers; thence exhausting most of the air from such containers and thence boiling said containers and contained alloy in boiling water for a short interval of time to anneal said contained alloy to the desired degree.

EDWARD L. CHOTT.